

# United States Patent Office.

KASSON FRAZER, OF SYRACUSE, NEW YORK.

*Letters Patent No. 96,217, dated October 26, 1869.*

## IMPROVED MODE OF PLATING, COATING, AND ORNAMENTING ARTICLES OF IRON AND STEEL.

The Schedule referred to in these Letters Patent and making part of the same

To all whom it may concern:

Be it known that I, KASSON FRAZER, of Syracuse, in the county of Onondaga, and State of New York, have invented a new and useful Mode of Plating, Coating, and Ornamenting Various Articles of Iron, such as harness-trimmings, buckles, snap-hooks, and other small wares made of wrought-iron, cast-iron, malleable iron, brass, and steel; and I hereby declare the following to be a full and exact description of the same.

The article to be treated is formed of a suitable useful or ornamental shape.

The figures to form the ornaments are made in relief in the ordinary manner, that is, by casting, stamping, or engraving.

After the article is formed, it is first japanned or coated with any suitable lacquer or varnish, such as will fully protect the article.

This process being well known need not be particularly described.

I next remove the japan or varnish by means of an emery-wheel or other proper abrading means, from the prominent parts of the article or the parts to which I wish to apply a plating of silver or other bright non-corrodible metal. This gives me a clear metallic surface, while the rest of the article remains covered by the lacquer or varnish.

I then coat the parts from which the japan or varnish has been removed with tin-solder or other metal, such as commonly used, uniting the non-corrodible metals, such as silver with iron. A number of these may be used, but I prefer tin-solder.

I next plate with sheet-metal by the ordinary silver close-plating process the parts which have been tinned or otherwise coated. This, with the usual burnishing, completes the article.

Having thus described my invention, What I claim, and desire to secure, by Letters Patent, is—

1. The herein-described method of plating and coating articles made as herein described, the said process consisting in first coating or varnishing, then removing the coating or varnish from the parts to be plated, and afterward plating the same, substantially as described.

2. The new article of manufacture made by the process herein described.

The above signed by me, this 2d day of October, 1869.

KASSON FRAZER.

Witnesses:

W. S. HUNTINGTON,  
PETER BURNS.